

April 16, 1935.

H. DREYFUS

1,997,633

MANUFACTURE OF ARTIFICIAL FILAMENTS OR THREADS

Filed April 4, 1929

FIG.2.



FIG.1.



Inventor  
HENRY DREYFUS

J. Seltzer and B. W. Lernson  
by  
Attorneys

## UNITED STATES PATENT OFFICE

1,997,633

MANUFACTURE OF ARTIFICIAL FILAMENTS  
OR THREADS

Henry Dreyfus, London, England

Application April 4, 1929, Serial No. 352,441  
In Great Britain April 10, 1928

5 Claims. (Cl. 18—8)

This invention relates to the manufacture of artificial silk and other filaments or threads from solutions of cellulose derivatives, for example, cellulose acetate or other cellulose esters or cellulose ethers, by dry-spinning or evaporative methods.

In accordance with the invention described in U. S. patent specification No. 1,602,125, artificial filaments or threads are produced by extruding a solution containing cellulose acetate or other cellulose derivative dissolved in a volatile solvent liquid through one or more jets or nozzles located in the upper part of a spinning chamber, leading the filaments or threads downwards through an atmosphere of warm or hot air or other gaseous evaporative medium within the spinning chamber, and winding the solidified filaments resulting from the evaporation of the volatile solvent liquid mechanically on apparatus located outside the chamber. The air or other gaseous evaporative medium is heated by suitable heating devices, and is preferably caused to flow in counter-current to the passage of the filaments. The filaments are associated into threads on their way to the winding device, and may be wound thereon either with or without twisting.

As explained in the above specification, the time during which the filaments are exposed to the evaporative influence of the heated air or other gas before issuing from the chamber must be such as to ensure that the volatile solvents are sufficiently evaporated and the filaments sufficiently solidified in their travel through the chamber. The necessary time of such exposure varies with the boiling points and quantity of the volatile liquids used in the spinning solutions, the denier of the filaments, and the temperature and speed of the current of air or other evaporative medium passing through the chamber.

Usually the period taken by the filaments in passing from the jets or nozzles to the point at which they emerge from the chamber is only very short, so that the filaments need only travel a relatively short distance in the chamber.

The present invention is based on the fact that, for certain purposes, advantage is presented when the path traversed by the filaments during their passage from the jets or nozzles to the point at which they leave the chamber is from 3 to 6 yards or more in length.

According to the invention, a process for the production of filaments or threads from solutions of cellulose acetate or other cellulose derivative comprises extruding the solutions downwards into a spinning chamber, causing the filaments

or threads to follow a path of 3 to 6 yards or more in length through the evaporative medium in the chamber, and winding the solidified filaments or threads mechanically outside the chamber.

It is found that, under any given set of spinning conditions, which will, of course, vary with the denier spun and the spinning solutions employed, the filaments obtained in accordance with the present invention display a remarkable regularity as regards their physical characteristics.

It is also of interest to note that owing to the length of the path traversed by the filaments within the spinning chamber, it is possible to secure complete or substantially complete removal of the volatile solvent before the filaments issue from the spinning chamber. In this way, loss of volatile solvent by evaporation outside the chamber can be prevented. This result is achieved without decreasing the concentration of the solvent vapours in the air or other evaporative medium which is led from the spinning chamber to the recovery plant, which is thus enabled to work under the optimum conditions of efficiency.

In one form of apparatus constructed in accordance with this invention, the filaments are led from spinning jets or nozzles in the upper part of the chamber to a point below the point at which the filaments emerge from the chamber, and are led back in an upward direction to the point of exit, the filaments thus following a more or less tortuous path in the chamber. In this case, the lower part of the spinning chamber is fitted with a guide or roller or similar device, around which the filaments are caused to pass on their way to the point at which they leave the chamber. The distance between the jets or nozzles and the guide, roller or similar device around which the filaments pass, may be shorter than the path of the filaments in spinning cells as heretofore constructed, but is preferably of the same or of greater length. The total distance from the jets or nozzles to the guide, roller or like device, and from the guide, roller or like device to the point of exit for the filaments must not be less than 3 yards, and is preferably 4 or 5 or even 6 yards or more.

Other methods of carrying out the invention will readily suggest themselves. For instance, it is possible to extend the foot of the spinning cell or chamber in a lateral or a horizontal direction, while keeping its height the same as that at present employed, the filaments being caused to pass around a guide, roller or like device in

the lower part of the spinning cell and thence in a lateral direction through the lateral extension thereof.

Instead of or in addition to employing a guide, 5 roller, or other device to divert the filaments in the spinning cells or chambers so as to cause them to follow paths of 3 to 6 yards or more from the jets or nozzles to the points at which they leave the cells or chambers, the height of the 10 cells or chambers may be increased to such an extent that the faces of the jets or nozzles are from 3 to 6 yards or more or much more above the point at which the filaments issue from the chamber.

15 In apparatus in which the filaments are caused to pass around a guide, roller or like device within the spinning cell, the arrangement may be such as to provide for a separate control of the extent to which the filaments are drawn out or stretched before they reach the guide, 20 roller or like device and the extent to which they are drawn out after they have passed said device. For example, the roller may be driven at an appropriate speed, the filaments being if necessary lapped around the roller, so that the superficial speed of the roller is imparted to the filaments.

25 The invention is applicable to the production of filaments of any desired characteristics, 30 whether round, or roundish, ribbon-like, voluminous, or cellular or tubular in structure. While the invention is particularly applicable to the production of filaments or threads having a basis of cellulose acetate, it may also be 35 used for the manufacture of filaments or threads from solutions containing cellulose formate, propionate or butyrate, or thiocarbamic or alkoxy-alkacetyl esters of cellulose, or methyl, ethyl or benzyl cellulose, or the corresponding 40 condensation products of cellulose and glycols or other polyhydric alcohols, or other substitution derivatives of cellulose that are capable of being formed into artificial filaments or threads by evaporative or dry-spinning methods.

45 Referring to the accompanying drawing Figs. 1 and 2 illustrate apparatus for carrying out the process according to the invention, alternative methods for causing the filaments or threads to follow paths of 3 or more yards in length 50 being indicated.

55 In Fig. 1, 1 is a spinning nozzle arranged at the upper end of a cell or chamber 2. Evaporative medium, such as air, enters the cell 2 by the inlet 3, the medium being heated on entering 60 the cell, or heated inside the cell by means such as the heating pipes 4. The filaments 5 extruded from the nozzle 1 are solidified in their passage through the evaporative medium and leave the cell in the form of a thread 6 through an opening 7.

65 The filaments 4 in their passage through the cell travel to a point below the level of the opening 7, and a guide roller 8 is arranged near the bottom 9 of the cell to receive the threads and enable them to return in an upward direction to the opening 1. The length of the cell and the position of the roller 8 are such that the more or less tortuous path traversed by the filaments from the nozzle 1 to the roller 8 and from the 70 roller to the opening 7 is at least 3 yards, and preferably 4 yards or more in length.

75 In addition to the advantage of high solvent recovery offered by the path of 3 yards or more during which the filaments are exposed to the evaporative medium, the evaporative power of

the medium may be enhanced by the employment of the collector devices described in U. S. patent application Serial No. 236,448 filed 29th November, 1927. One such device is shown in the figure and consists of a cylindrical tube 10 through which the evaporative medium has to pass on its way to a suction draw-off 11, the medium being thereby constrained to pass through the immediate vicinity of the nozzle 1. The draw-off 11 comprises an annular pipe perforated on its underside with a series of holes 12 and disposed coaxially with the pipe 13 that supplies the spinning solution to the nozzle 1. The draw-off 11 is arranged somewhat above the level of the nozzle and assists the collector device 10 in bringing the evaporative medium through the neighbourhood of the nozzle. A tube 14 connects the draw-off 11 to a pipe 15 that communicates through a valve 16 with a header 17, the valve 16 being controlled by a handle 18 20 to regulate the flow of the evaporative medium in conjunction with a flow-meter 19 connected to the pipe 15, as is described in U. S. patent specification No. 1,541,104.

25 Instead of employing the guide roller 8 as is shown in Fig. 1 to ensure that the filaments follow a path of at least 3 yards in length, the height of the nozzle 1 above the opening 7 may be increased as is shown in Fig. 2 to at least 3 yards, and preferably 4 yards or more, and the 30 filaments may then be led directly from the nozzle 1 to the opening 7, the requisite length of path according to the invention being furnished by this disposition of the nozzle 1 and the opening 7. The last-mentioned arrangement does not 35 require the bottom of the cell 2 to be much below the level of the opening 7, suitable relative positions of the bottom 9 and the inlet 3 for the evaporative medium being shown in Fig. 2.

40 In both figures, the thread 6 after leaving the cell 2 by the opening 7 passes over or round a feed roller 20 and proceeds to any suitable winding or a twisting and winding device, such as the cap-spinning device 21.

45 An inspection opening 22 is provided in the cell at about the level of the nozzle 1 to provide access to the nozzle. The tube 10 is preferably 50 slidably mounted in a funnel 23 so as to be readily adjustable, and also movable away from the nozzle. Heating means 24 may be provided immediately below the collector device 10.

55 The roller 8 may be positively driven in any convenient manner and may rotate at a speed higher than the speed of extrusion of the filaments, thereby stretching the filaments in their 60 passage from the nozzle 1 to the roller 8. The roller 20 is preferably positively driven and may still further stretch the filaments after they have left the roller 8.

65 It is to be understood that the foregoing details are merely given by way of illustration and that many variations may be made therein without departing from the spirit of the invention.

What I claim and desire to secure by Letters Patent is:—

1. A process for spinning artificial filaments or threads from solutions of cellulose acetate or other cellulose derivatives, said process comprising spinning the solutions into a current of evaporative medium secluded from the atmosphere, 70 causing the filaments or threads to follow a path of at least 3 yards in length through said evaporative medium, withdrawing said filaments or threads from said evaporative medium, and finally 75 winding the filaments or threads.

2. Apparatus for the spinning of artificial filaments or threads by the evaporative method, comprising a spinning chamber, at least one spinning nozzle in said chamber, winding apparatus located outside the chamber, an outlet from the chamber, and guide means for the filaments or threads in the chamber below the level of said outlet, the apparatus presenting a path from the spinning nozzle round the guide means to the 5 said outlet at least 3 yards in length.
3. In the spinning of artificial filaments from solutions of derivatives of cellulose by extruding the filaments into a current of heated gaseous medium secluded from the atmosphere, the step 10 of causing the filaments to pursue a tortuous extended path of at least three yards in length through said heated medium, withdrawing said filaments or threads from said evaporative medium, and finally winding the filaments or 15 threads.
4. Apparatus for the spinning of artificial filaments by the evaporative method, said apparatus comprising at least one spinning nozzle and a spinning chamber adapted to contain said nozzle and provided with an outlet for the filaments extruded into the chamber, said chamber being further adapted to afford to the filaments between said nozzle and said outlet an extended path of at least three yards in length. 5
5. Apparatus for the spinning of artificial filaments by the evaporative method, said apparatus comprising at least one spinning nozzle and a spinning chamber adapted to contain said nozzle provided with an outlet for the filaments extruded into the chamber, and guide means within 10 said chamber adapted to conduct the filaments between said nozzle and said outlet along an extended path of at least three yards in length. 15

HENRY DREYFUS. 20